

## UNITED STATES PATENT OFFICE

2,060,186

## DYEING OF ACETATE ARTIFICIAL SILK

Friedrich Felix, Basel, Max Bommer, Riehen,  
near Basel, and Wilhelm Huber, Basel, Switzerland, assignors to the firm Society of Chemical Industry in Basle, Basel, Switzerland

No Drawing. Original application October 11, 1933, Serial No. 693,219. Divided and this application June 18, 1934, Serial No. 731,216. In Switzerland October 15, 1932

## 2 Claims. (Cl. 8-5)

This application is a division of our application for patent Serial No. 693,219, filed in the United States on October 11, 1933, and in Switzerland on October 15, 1932.

5 It is known that acetate artificial silk can be dyed by means of feebly basic, sparingly soluble or insoluble dyestuffs. While a large number of such dyestuffs dye acetate artificial silk only feeble or matt tints, the number of dyestuffs 10 capable of dyeing such silk in deep full tints is comparatively small. The number cannot be increased directly by introducing substituents into the molecule of the dyestuff, since very frequently the enlargement of the molecule is associated 15 with a strong diminution of the affinity of the dyestuff for acetate artificial silk.

The present invention relates to a composition of matter and to a process for dyeing acetate artificial silk in which the dyeing is conducted 20 with a composition of matter consisting of a mixture of a feebly dyeing dyestuff with a similarly constituted dyestuff. The term "similarly" comprises the homologous, analogous and isomeric dyestuffs having a somewhat similar shade. Such a composition of matter presents an increased affinity for the fiber which is quite considerable and makes it possible to use products which hitherto have had no practical value. The dyestuff of low affinity becomes more readily 25 adsorbed when it is mixed with a dyestuff which in itself has a practically sufficient affinity for acetate artificial silk. In this manner the affinity of the already useful acetate artificial silk dyestuff may be improved. Furthermore, it is 30 possible by use of such a composition of matter to shift the color tint of the dyeing in a desired manner in one or the other direction without introduction of substituents into the dyestuff molecule of the dyestuff of good affinity, which 35 introduction, as already stated, may affect the degree of affinity of the dyestuff in an unfavourable manner.

The compositions of matter of the present invention may be made by adding to the components of a dyestuff during its manufacture a homologue, isomeride or analogue thereof, or by dissolving the finished dyestuffs in a common solvent and precipitating them together in a finely divided state, or by finely grinding together the finished dyestuffs, or by adding the previously finely subdivided dyestuffs to the same dye-bath.

The process is applicable to all classes of dyestuffs usual in the acetate artificial silk dye-house. It finds a special application in the case

of dyestuff preparations from azo-dyestuffs and in the present case from aminoanthraquinones. When the preparation is to be made from an azo-dyestuff there may be added to the coupling component or to the diazo-component or to both, 5 a homologue, isomeride or analogue thereof, and the mixture of dyestuffs may thus be made directly, or the finished azo-dyestuffs may be mixed with each other by fine grinding or may be added to the same dye-bath. The procedure is similar 10 in making dyestuff preparations from aminoanthraquinones; in this case a good intermixture may be achieved, among other methods, by dissolving the homologues, isomerides or other analogous dyestuffs in the same solvent and precipitating the mixture in finely divided form in 15 some suitable manner.

The following examples illustrate the invention, the parts being by weight:—

## Example 1 20

6 parts of 1-amino-4-anilidoanthraquinone and 4 parts of 1-amino-4-para-toluididoanthraquinone are introduced into 100 parts of sulfuric acid of 98 per cent. strength at 0-10° C. and the mass is 25 stirred until dissolution is complete. The solution is poured upon ice, filtered and washed until neutral. If the dyestuff thus obtained is brought into a suitable form by grinding with a dispersing agent there is obtained a preparation 30 which dyes acetate artificial silk intensely blue tints, whereas the dyeings obtained with the individual dyestuffs are less intense. The intimate mixture of 1-amino-4-para-toluididoanthraquinone and 1-monomethylamino-4-anilidoanthraquinone 35 also dyes acetate artificial silk blue, as also the ternary mixture of 1-amino-4-anilidoanthraquinone, 1-amino-4-para-toluididoanthraquinone and 1-monomethylamino-4-anilidoanthraquinone. 40

## Example 2

6 parts of a paste of 10 per cent. strength of 1-amino-4-anilidoanthraquinone and 4 parts of a paste of 10 per cent. strength of 1-amino-4-para-toluididoanthraquinone are together stirred with 45 about the same total weight of a soap solution of 6 per cent. strength at about 50° C. and the whole is diluted with lukewarm water to 300 parts. 10 parts of acetate artificial silk are now entered, the temperature of the bath is raised within 3/4 50 hour to 75-80° C. and the goods are handled for about 3/4 hour at this temperature. Rinsing and drying follow. The acetate artificial silk is dyed intensely blue.

A greenish blue is obtained by the use of a 55

mixture of 7.5 parts of 1-amino-4-(4'-amino)-phenylaminoanthraquinone and 2.5 parts of 1-methylamino - 4 - (4'-hydroxy) - phenylaminoanthraquinone.

5 What we claim is:—

1. A dyeing composition consisting of a mixture of at least two acetate artificial silk dyestuffs, of which at least one has a poor affinity for acetate artificial silk, selected from the group of the products of the general formula

15



20

in which R<sub>1</sub> stands for a member of the group consisting of hydrogen and methyl, and R<sub>2</sub> stands for a member of the group consisting of hydrogen, methyl, hydroxyl and amino.

25 2. A process of dyeing acetate artificial silk

wherein the operation is conducted with a composition of matter, brought into a fine state of dispersion, consisting of at least two acetate artificial silk dyestuffs, of which at least one has a poor affinity for acetate artificial silk, selected 5 from the group of the products of the general formula



10

15

in which R<sub>1</sub> stands for a member of the group consisting of hydrogen and methyl, and R<sub>2</sub> stands for a member of the group consisting of hydrogen, methyl, hydroxyl and amino. 20

FRIEDRICH FELIX.  
MAX BOMMER.  
WILHELM HUBER.

25